

Patented Oct. 6, 1925.

1,555,959

# UNITED STATES PATENT OFFICE.

ANDRÉ ANGELO FRESNEAU, OF AUBERVILLIERS, FRANCE.

## LIGHT ALLOY AND PROCESS OF MANUFACTURE OF THE SAME.

No Drawing.

Application filed March 6, 1924. Serial No. 697,395.

To all whom it may concern:

Be it known that I, ANDRÉ ANGELO FRESNEAU, citizen of the French Republic, residing at Aubervilliers, Seine, in the 5 French Republic, have invented new and useful Improvements in Light Alloys and Processes of Manufacture of the Same, of which the following is a specification.

A certain number of quaternary alloys of 10 light weight are already known, such as duralumin which is composed of aluminium, copper, manganese and magnesium, the A alloy composed of aluminium, copper, zinc, and silicon, the E alloy consisting of copper, 15 zinc, magnesium and manganese, and the Y alloy composed of aluminium, copper, nickel and magnesium. These light alloys have in all cases a great strength, this being variable according as the metal is rolled, drawn, cast 20 or forged.

My invention has for its object a light alloy formed of aluminium, copper, nickel, zinc and magnesium and having approximately the following percentage composi- 25

tion:

|           |       |
|-----------|-------|
| Aluminium | 93.32 |
| Copper    | 3.4   |
| Nickel    | 1.0   |
| Zinc      | 1.78  |
| Magnesium | 0.5   |

For the manufacture of the said alloy, I proceed as follows: I first prepare a ternary alloy composed of:

|        |      |
|--------|------|
| Copper | 54.5 |
| Nickel | 16.5 |
| Zinc   | 29.0 |

The melted alloy is well stirred, and is then deoxidized by adding 2 percent of baryta.

40 I then take 6.5 kilograms of the melted and deoxidized alloy and pour the same into a crucible containing 100 kilograms of aluminium in fusion. The mixture is well stirred, and after about 5 minutes I add 45 500 grams of magnesium. I then add, while continuing the stirring, 2 kilograms of caustic soda which has been previously dried at a red heat. The soda renders the alumina soluble and the bath is thus made 50 fluid; the latter is skimmed off and is then ready for casting, which is carried out at about 700° C., this temperature being variable by some 15° either way.

55 The resulting alloy is remarkably light, its density being in fact about 2.9, but at the same time it possesses great strength.

After 1 1/4 hours' thermic treatment at about 530° C., followed by a rapid immersion in water at about 25° (within 5° more or less) to obtain a complete cooling, and 60 a subsequent tempering in boiling water at 100°, my alloy has the following tensile strength:

|                                    |                     |
|------------------------------------|---------------------|
| 17 to 19 kgs. per m/m <sup>2</sup> | for cast metal,     |
| 45 to 50 kgs. per m/m <sup>2</sup> | for drawn metal, 65 |
| 42 to 48 kgs. per m/m <sup>2</sup> | for rolled metal,   |
| 46 to 52 kgs. per m/m <sup>2</sup> | for forged metal.   |

The corresponding elongations are:

|                                             |                          |
|---------------------------------------------|--------------------------|
| 8 to 11 per cent                            | for cast metal, 17 to 22 |
| per cent for drawn metal, 17 to 22 per cent | 70                       |
| for rolled metal, 16 to 22 per cent         | for forged metal.        |

It should also be observed that the heating and cooling curves for the said alloy show no particular features nor critical 75 points.

Obviously, I may vary the proportions of the constituent metals of the said alloy to a slight degree, without departing from the 80 scope of the invention.

Having now described my invention, what I claim as new and desire to secure by Letters Patent is:

1. A metal alloy the composition whereof is substantially: aluminium 93.3, copper 3.4, 85 nickel 1, zinc 1.8 and magnesium 0.5.

2. The process of manufacture of a metal alloy containing aluminium, copper, nickel, zinc and magnesium which consists in preparing a ternary alloy containing the whole 90 amount of copper, nickel and zinc, pouring said melted ternary alloy into the melted mass of aluminium and then adding the desired quantity of magnesium.

3. The process of manufacture of a metal alloy containing aluminium, copper, nickel, zinc and magnesium which consists in preparing a ternary alloy containing the whole amount of copper, nickel and zinc, pouring said melted ternary alloy into the melted 100 mass of aluminium, then adding the desired quantity of magnesium, adding subsequently anhydrous caustic soda and skimming the slag off the bath.

4. The process of manufacture of a metal alloy the composition whereof is substantially: aluminium 93.3, copper 3.4, nickel 1, zinc 1.8 and magnesium, which consists in preparing a ternary alloy containing the whole amount of copper, nickel and zinc, 105 pouring said melted ternary alloy into the melted mass of aluminium, then adding the 110

corresponding quantity of magnesium and casting the alloy thus obtained at a temperature substantially equal to 700° C.

5. The process of manufacture of a metal alloy containing aluminium, copper, nickel, zinc and magnesium which consists in preparing a ternary alloy containing the whole amount of copper, nickel and zinc, adding

baryta to said ternary alloy for deoxidizing the same, pouring said deoxidized ternary 10 alloy into the melted mass of aluminium and then adding the desired quantity of magnesium.

In testimony whereof I have signed my name to this specification.

ANDRÉ ANGELO FRESNEAU